

- [54] SILVER HALIDE PHOTOGRAPHIC MATERIAL CONTAINING A HYDROXYAZAIDENE AND A CARBOXYL SUBSTITUTED 1,2-DITHIOLANE AS STABILIZING COMBINATION
- [75] Inventors: Susumu Kondo; Tadao Sakai; Reiichi Ohi; Mitsunori Sugiyama, all of Kanagawa; Mitsuo Numata, Osaka, all of Japan
- [73] Assignee: Fuji Photo Film Co. Ltd., Kanagawa, Japan
- [22] Filed: Mar. 23, 1973
- [21] Appl. No.: 344,399
- [30] Foreign Application Priority Data  
Mar. 29, 1972 Japan..... 47-31434
- [52] U.S. Cl..... 96/107, 96/108, 96/109  
[51] Int. Cl..... G03c 1/28, G03c 1/34  
[58] Field of Search..... 96/107, 108, 109

- [56] References Cited  
UNITED STATES PATENTS
- |           |         |                          |        |
|-----------|---------|--------------------------|--------|
| 2,728,668 | 12/1955 | Mochel .....             | 96/109 |
| 2,948,614 | 8/1960  | Allen et al. ....        | 96/109 |
| 3,128,186 | 4/1964  | Corben et al. ....       | 96/109 |
| 3,732,104 | 5/1973  | Vandenabeele et al. .... | 96/109 |

Primary Examiner—Norman G. Torchin  
Assistant Examiner—Won H. Louie, Jr.  
Attorney, Agent, or Firm—Sughrue, Rothwell, Mion,  
Zinn & Macpeak

[57] ABSTRACT  
A silver halide emulsion layer in a photographic material which contains at least one triazaindene, tetraza-indene or a pentazaindene having at least one hydroxy group and at least one compound having a 1,2-dithiolane or a 1,2-dithiane ring exhibits lower fogging but substantially no reduction in desirable photographic characteristics.

15 Claims, No Drawings

**SILVER HALIDE PHOTOGRAPHIC MATERIAL  
CONTAINING A HYDROXYAZAIDENE AND A  
CARBOXYL SUBSTITUTED 1,2-DITHIOLANE AS  
STABILIZING COMBINATION**

**BACKGROUND OF THE INVENTION**

1. Field of the Invention

The present invention relates to a silver halide photographic light-sensitive material and, more particularly, to a silver halide photographic light-sensitive material designed to show lower fogging and show reduced variation in photographic characteristics during storage without a reduction in sensitivity.

2. Description of the Prior Art

As methods to enhance the sensitivity of a silver halide emulsion, there have been known sulfur sensitization, noble metal sensitization, reduction sensitization, sensitization with a selenium compound and the like. These sensitizing methods are usually referred to as chemical sensitizations. The sensitizing method with alkylene oxide or polyalkylene glycols is also well known. It is further known to suitably combine two or more of these sensitizing methods to thereby obtain a required photographic sensitivity.

However, when these sensitizing methods are employed, fogging is liable to increase though there is recognized a remarkable increase in photographic sensitivity. Therefore, it is necessary to lower such fogging. A number of compounds have been suggested for this purpose.

Such compounds are, in general, called "anti-fogging agents" among those skilled in the art and, in some cases, are referred to as "stabilizing agents." These so-called anti-fogging agents have the common property of lowering the fogging of photographic emulsions but, at the same time, possess the defect of reducing photographic sensitivity or other photographic characteristics, e.g., gamma. Accordingly, the anti-fogging agents have so far been used with some unavoidable loss of sensitivity. Therefore, a method to lower the fogging alone while maintaining the inherent photographic sensitivity has been eagerly sought.

**SUMMARY OF THE INVENTION**

A primary object of the present invention is to provide a silver halide photographic light-sensitive material wherein fogging is sufficiently lowered without a reduction in sensitivity.

Another object of the invention is to provide a silver halide photographic light-sensitive material wherein the increase in fogging during storage is lowered.

A further object of the invention is to provide a silver halide photographic light-sensitive material undergoing less variations in sensitivity or gamma value during storage.

Compounds having a 1,2-dithiolane ring or a 1,2-dithiane ring are known as an anti-fogging agent for silver halide photographic emulsions. However, while these compounds depress fogging, they have the defect that, similarly to other anti-fogging agents, they degrade sensitivity and other photographic characteristics. The inventors have now found that the defects of the compounds having a 1,2-dithiolane ring or a 1,2-dithiane ring, such as a reduction in sensitivity, can be

removed by the combined use of such compounds and one or more azaindenes.

This fact is quite surprising taking into consideration that azaindenes are well known as an anti-fogging agent or a stabilizing agent among those skilled in the art, i.e., such a fact could not be anticipated at all from the conventional common knowledge that in general anti-fogging or stabilizing agents reduce the sensitivity though they have the action of depressing fogging as is described above.

**DETAILED DESCRIPTION OF THE INVENTION**

The present invention relates to a photographic material comprising a support having thereon a silver halide emulsion layer containing at least one compound having a 1,2-dithiolane ring or a 1,2-dithiane ring (hereinafter referred to as "compound A") and at least one of triazaindenes, tetraazaindenes or pentazaindenes, which have at least one hydroxy group (hereinafter referred to as "compound B").

As preferred examples of compound A used in the invention, there are illustrated the compounds represented by the following formula;



wherein X represents a divalent (hydrocarbon) residue having 1 - 6 carbon atoms, R represents a carboxylic acid group, a carboxylic acid salt group, a carboxylic acid ester group, or a carboxylic acid amide group, m represents 2 or 3, and n represents 0 or 1.

As preferred examples of X in general formula (I), there are methylene, ethylene, propylene, butylene, hexylene, etc.

As examples of preferred carboxylic acid salts there are alkali metal salts (e.g., sodium salts, potassium salts, etc.), alkaline earth metal salts (e.g., calcium salts, barium salts, etc.), ammonium salts, amine salts (e.g., methylamine salts, ethylamine salts, ethanolamine salts, etc.) and the like. The salts used are, of course, cation salts with the carboxylic acids.

Examples of preferred carboxylic acid esters are esters with a  $\text{C}_1 - \text{C}_{12}$  alkyl group or a phenyl group, and the like.

Examples of preferred carboxylic acid amides are carboxylic acid amide and carboxylic acid amide substituted by a  $\text{C}_1 - \text{C}_{12}$  alkyl group or by a phenyl group, and the like.

Additionally, in the above-illustrated general formula (I), when m represents 2, a dithiolane ring is formed and, when m represents 3, a dithiane ring is formed.

Compound A used in the invention is structurally characterized by containing a dithiolane ring or a dithiane ring, and exerts the action of lowering fogging of silver halides due to this structural feature. Therefore, compound A used in the invention is not particularly limited to that represented by the foregoing general formula (I), and any compound having a dithiolane or a dithiane ring may be used.

The compounds represented by the foregoing general formula (I) may be synthesized according to known processes, e.g., described in "Journal of the American Chemical Society," 76, pp. 1,828 - 1832 (1954).

The following are typical compounds represented by general formula (I) useful in the present invention.



15 Compound B used in the invention includes triazaindenes, tetrazaindenenes and pentazaindenenes which have at least one hydroxy group attached to a carbon atom which forms the azaindene ring. The preferred substitution point(s) for the OH group(s) is the 5- and/or 7-position on the azaindene ring, but this is not limitative. These compounds may further contain substituents in addition to the hydroxy group, and such are included within the terms triazaindenes, tetrazaindenenes and pentazaindenenes in the specification and claims. As specific examples of such substituents, there are illustrated a halogen, an alkyl group having 1 - 17 carbon atoms, an aralkyl group, an aryl group, an alkoxy group having 1 - 18 carbon atoms, a carboxyl group, an alkoxy carbonyl group having 1 - 18 carbon atoms, an aminocarbonyl group, a cyano group, a group forming a hydrocarbon ring together with the adjacent carbon atoms (See for example, compounds B-12, B-14, where a saturated ring is formed; the adjacent carbon atoms are bincinal carbon atoms which form the azaindene ring), and the like.

and the like.

In the present invention, the presence of any special substituent(s) on the azaindene ring other than the hydroxy group is rather immaterial and any substituent(s) excepting those such as a nitro group or mercapto group which adversely affect the photographic properties, such as sensitivity and fog, of the light-sensitive emulsion can be present. All such substituted azaindenes are to be construed as within the scope of the present invention.

Compound B is characterized by containing an azaindene ring having at least one hydroxy group, and may contain substituents other than are described above.

Compound B may be synthesized according to known processes, e.g., described in "Chemical and Pharmaceutical Bulletin," 6, pp. 583 - 586 (1958), or *ibid.*, 10, pp. 612 - 620 (1962).

Typical useful examples of compound B are as follows.





The amounts of compound (A) and compound (B) added vary depending upon the presence of additives to the emulsion, such as a sensitizing agent. In general, greater amounts of a sensitizing agent causes higher fog density, thus, greater amounts of the compounds are needed. In general, compound (A) is suitably added in an amount of from about 0.0005 g to about 5 g and compound (B) from about 0.005 to about 50 g, per 1 mol of silver halide contained in the emulsion. Preferably, compound (A) is added in an amount of from about 0.005 to 0.5 g, compound (B) from about 0.05 to 5 g, same basis as above. The optimal amount can be determined by the preliminary test well known by those skilled in the art, i.e., a series of runs, wherein the amount of the compounds is varied.

As will be appreciated by one skilled in the art, one can use one or more different compounds (A) in combination with one or more different compounds (B). In this case of course, the total amount of the different compounds suitably falls within the ranges recited above.

These compounds are added to a silver halide emulsion advantageously as a solution. As a suitable solvent, organic solvents which exert no detrimental effect on a photographic emulsion, such as lower alcohols and ketones, as well as water, can be used.

In general, a silver halide photographic light-sensitive material is produced via the following steps; (1) preparation and weighing of starting materials for the production of emulsion; (2) emulsification; (3) first ripening or physical ripening; (4) removal of water-soluble salts; (5) second ripening or chemical ripening; and (6)

coating of the emulsion. (For example, see "Making and Coating Photographic Emulsions," pp. 17 - 22, issued by Focal Press Co.)

According to the present invention, compound (A) and compound (B) may effectively be added to an emulsion during production of the silver halide emulsion (i.e., in the above-described steps (1) to (5)) or immediately before coating the emulsion. A particularly preferred stage of the addition is between the second ripening step and the coating step.

As the silver halide for the photographic emulsion in the present invention, any of the known ones such as silver chloride, silver bromide, silver chlorobromide, silver bromoiodide, silver chloroiodide, silver chlorobromoiodide and the like can be used. In addition, halogen conversion-type silver halide grains as described in British Pat. No. 635,841 may also be used effectively.

As the binder for the silver halide, any hydrophilic colloid applied to usual silver halide emulsions may be used. For example, gelatin, albumin, gum arabic, agar-agar, cellulose derivatives (e.g., carboxycellulose alkyl esters, hydroxyethyl cellulose, carboxymethyl-hydroxyethyl cellulose, etc.), synthetic resins (e.g., polyvinyl alcohol, polyvinyl pyrrolidone, etc.), and the like are merely a small sampling of those hydrophilic colloids which can be used in the present invention.

The generally used ratio of silver halide : binder is 1 : about from 0.1 to 20. A preferred particle size for the silver halide is from about 0.05 to about 5 microns. Neither of these ranges are limitative, and they can be varied in a manner known to the art.

To the photographic emulsions used in the invention may be added, in a manner known to the art, compounds containing group I elements such as rubidium, cesium, copper, silver, gold, etc., group II elements such as magnesium, strontium, zinc, cadmium, mercury, etc., group VIII elements such as iron, cobalt, nickel, ruthenium, rhodium, palladium, osmium, iridium, platinum, etc., in order to adjust the photographic characteristics of the emulsion.

Also, the photographic emulsion can be subjected to chemical ripening with active gelatin or with the use of a sulfur compound in a manner as described in U.S. Pat. Nos. 1,574,944; 1,623,499 or 2,410,689.

The photographic emulsion can be chemically sensitized with gold salts such as are described in U.S. Pat. No. 2,399,083; with reducing agents such as the stannous salts described in U.S. Pat. No. 2,487,850; reducing agents such as the polyamines described in U.S. Pat. No. 2,521,925; with bis(beta-aminoethyl)sulfides and the water-soluble salts thereof described in U.S. Pat. No. 2,521,926; with compounds containing a labile selenium atom as described in U.S. Pat. Nos. 3,297,446; 3,297,447 and 3,442,653; can be sensitized by the addition of polyalkylene glycols as described in U.S. Pat. Nos. 2,423,549 and 2,441,389; or with various derivatives of alkylene oxides as described in U.S. Pat. No. 2,240,472 and British Pat. No. 443,559.

The above-described photographic emulsion may, of course, be spectrally sensitized with a cyanine or merocyanine dye.

The hydrophilic colloid used in the photographic light-sensitive material of the invention is advantageously hardened by the generally used hardeners of the aldehyde series, methylol series, 1,4-dioxane series,

aziridine series, isoxazole series, carbodiimide series, active halogen series, active vinyl series, etc.

The light-sensitive photographic material of the invention can be either a black-and-white photographic material which provides a final image comprising metallic silver, or a color photographic material which provides a final image comprising dyes.

In the case of color photographic light-sensitive materials, all of the ketomethylene yellow dye-forming 10 couplers can advantageously be used. Typical examples thereof are couplers of the benzoylacetanilide series, pivalylacetanilide series, etc. Further, all of the magenta dye-forming couplers of the pyrazolone series, indazolone series, etc., can advantageously be used. In 15 addition, all of the cyan dye-forming couplers of the phenol series, naphthol series, etc., can advantageously be used. These couplers may contain a coupling-off group at the active carbon atom positioned at the coupling site. Those couplers rendered nondiffusible with 20 a ballast group are preferred. With respect to these couplers, a great number of ballasted compounds are well known.

These dye-forming couplers can be dispersed in a hydrophilic colloid in any known manner. They can advantageously be dispersed with the use of a coupler solvent as described in U.S. Pat. No. 2,322,027, etc.

The photographic light-sensitive material of the invention can contain a plasticizer such as glycerin, a coating aid such as saponin, polyethylene glycol monolauryl ether, etc., a lubricating agent such as a silicone resin, paraffin, etc., a matting agent such as starch, titanium dioxide, a silicate, etc., a water-soluble azo dye, polymethine dye, diphenylmethane dye, etc., a brightening agent of the styrene series, triazine series, oxazole series, coumarin series, etc., antistatic agents such as the ionic polymers described in U.S. Pat. No. 2,861,056, and antioxidants such as hydroquinone derivatives, ascorbic acid, etc.

In addition, the photographic light-sensitive material of the invention can contain ultraviolet ray-absorbing agents such as Michler's diketone sulfonic acid, benzotriazole, etc., or may contain colloidal silver, carbon black or the like to prevent static marks.

As the support advantageously used in the photographic light-sensitive material of the invention, there are cellulose ester films such as cellulose nitrate, cellulose acetate, etc., polyester films such as polyethylene terephthalate films, etc., polyvinyl chloride films, polystyrene films, polycarbonate films, baryta paper and aliphatic polymer laminated paper.

The photographic light-sensitive material of the invention may further comprise an antihalation layer containing colloidal silver, carbon black dye, etc., or a filter layer.

The photographic light-sensitive material of the invention can be processed in any known manner, e.g., with black-and-white developers as are commonly used, e.g., an alkali solution containing a developing agent such as a hydroxybenzene, aminobenzene, aminophenol, etc., which may contain a sulfite, carbonate, bisulfite, bromide, iodide, etc. of an alkali metal. Other useful black-and-white developing agents are described, for example, in "The Theory of the Photographic Process," 3rd Edition, pp. 278 - 331, issued by MacMillan Co.

Color developers as are commonly used in the art can also be used in the present invention, i.e., any alkaline

aqueous solution containing a color-developing agent. As the color-developing agents, all known dye-forming aromatic primary amine developers such as phenylenediamines (e.g., N,N-diethyl-p-phenylene-diamine, N-ethyl-N-hydroxyethyl-p-phenylenediamine, N-ethyl-N-hydroxyethyl-2-methyl-p-phenylenediamine, N-ethyl-beta-N-methanesulfonamidoethyl-3-methyl-4-aminoaniline, N,N-diethyl-2-methyl-p-phenylenediamine, and the sulfonates, hydrochlorides and sulfites thereof, etc.) can be used. The color developer may further contain generally used additives such as a sulfite, carbonate bisulfite, bromide or iodide of an alkali metal, benzyl alcohol and the like.

As other processing solutions, e.g., a bleaching solution, a fixing solution, a stabilizing solution, etc., ones known in the art may advantageously be used. These processing solutions may be used in combinations of two or more of them, e.g., as a bleach-fixing solution, a fix-stabilizing solution or a bleach-fixstabilizing solution.

Such solutions are well known in the art, and any of such known solutions are useful. A bleaching solution contains a silver oxidizing agent(s), e.g., water-soluble ferricyanides, a simple water-soluble ferric, cupric or cobaltic salt, and complex salts of an alkali metal and polyvalent cations with an organic acid. Typical examples of the polyvalent cations are ferric ions, cobaltic ions, cupric ions, etc. Typical examples of the organic acids are ethylene diamine tetraacetic acid, nitrilotriacetic acid, etc. A fixing solution contains a silver halide solvent(s) for example, a water-soluble thiosulfate, water-soluble thiocyanate, etc. A stabilizer solution contains, of course, a stabilizer such as formaldehyde, citric acid, etc. Specific examples of these compounds are illustrated on U.S. Pat. No. 3,582,322.

In the silver halide emulsion in accordance with the present invention containing compound A and compound B, fogging alone is lowered without a reduction in sensitivity or the gamma value. In addition, the emulsion has the feature that less fog is formed and variations in sensitivity and the gamma value are lessened during storage.

30

35

40

0.01 percent aqueous potassium chloroaurate solution and the emulsion was chemically ripened at 60°C for 60 minutes.

After the completion of ripening, the resulting emulsion was divided into three equal portions, one of which was used as a control and to the remaining two of which were added, respectively, the compounds described in Table 1. Each of the thus obtained three emulsions was applied to a triacetate cellulose film support in a coated silver amount of  $2.5 \times 10^{-2}$  mol/m<sup>2</sup>, then dried.

The thus prepared samples were subjected to sensitometry in a known manner to compare the sensitivity, gamma value and fog density of each sample. Development was conducted at 20°C for 8 minutes using a developer having the following composition.

|                                |         |
|--------------------------------|---------|
| N-Methyl-p-aminophenol sulfate | 2.2 g   |
| Hydroquinone                   | 8.8 g   |
| Anhydrous sodium sulfite       | 96.0 g  |
| Anhydrous sodium carbonate     | 48.0 g  |
| Potassium bromide              | 5.0 g   |
| Water to make                  | 1 liter |

After development, each of the samples was immersed in a stopping bath at 20°C (2 percent acetic acid aqueous solution) for 30 seconds, washed for 1 minute with a running water, then fixed at 20°C for 8 minutes using a fixing solution having the following composition, washed for 5 minutes with running water, and dried.

|                          |         |
|--------------------------|---------|
| Sodium thiosulfate       | 250 g   |
| Anhydrous sodium sulfite | 15 g    |
| Boric acid               | 8 g     |
| Potash alum              | 15 g    |
| Sodium acetate           | 10 g    |
| Water to make            | 1 liter |

In addition, the three samples were subjected to an incubation test. After leaving each sample at 50°C and at 80 percent RH for 48 hours in the unexposed state, they were exposed and developed in the same manner as in the case of the fresh samples. The results obtained are shown in Table 1.

TABLE 1

| Compound | Added amount of compound per 1 mol of silver (mg) | Fresh                |      | Incubated |                      |
|----------|---------------------------------------------------|----------------------|------|-----------|----------------------|
|          |                                                   | Relative sensitivity | amma | Fog       | Relative sensitivity |
| Control  | None                                              | 100                  | 1.20 | 0.12      | 115                  |
| A - 5    | 65                                                | 85                   | 1.00 | 0.08      | 70                   |
| A - 5    | 65                                                | 98                   | 1.18 | 0.08      | 95                   |
| B - 3    | 350                                               |                      |      |           | 1.22                 |
|          |                                                   |                      |      |           | 0.07                 |

The present invention will now be described in greater detail by several non-limiting examples of preferred embodiments.

#### EXAMPLE 1

To 1,000 g of a light-sensitive gelatino silver bromo-iodide (1.2 mol percent iodide) emulsion (containing 0.8 mol silver) having an average silver halide diameter of 1.0 micron there were added 30 ml of 0.01 percent aqueous sodium thiosulfate solution and 15 ml of a

As is evident from Table 1, although compound A has the effect of lowering fogging, it reduces both the sensitivity and gamma at the same time. On the other hand, when compound A and compound B are used in combination, fogging can be prevented without reducing sensitivity and gamma. In addition, almost no variations in the photographic characteristics were observed under the conditions of high temperature and high humidity, and thus, it can be seen that the sample in accordance with the invention has an extremely stable preservability.

## EXAMPLE 2

A silver halide gelatin photographic emulsion (containing 0.06 mol silver per 100 g) comprising silver chlorobromide containing 25 mol percent chlorine subjected to second ripening with the use of sulfur compound and gold salt was prepared in the same manner as in Example 1.

After the completion of ripening, the resulting emulsion was divided into 4 equal portions. One of them was used as a control, and to the remaining 3 portions were added, respectively, the compounds described in Table 2. Each of the resulting 4 emulsions was applied to a paper support having coated on both sides thereof polyethylene containing dispersed therein white titanium dioxide, in a coated silver amount of  $1.9 \times 10^{-2}$  mol/m<sup>2</sup>, then dried.

The thus prepared samples were subjected to sensitometry in a known manner to compare the sensitivity, gamma value and fog density of each sample. Development was conducted at 20°C for 2 minutes using a developer having the following composition.

|                                |           |    |
|--------------------------------|-----------|----|
| N-Methyl-p-aminophenol sulfate | 3.1 g     | 25 |
| Hydroquinone                   | 12.0 g    |    |
| Anhydrous sodium sulfite       | 45.0 g    |    |
| Anhydrous sodium carbonate     | 67.5 g    |    |
| Potassium bromide              | 1.9 g     |    |
| Water to make                  | 2 liters. |    |

After development, each of the samples was processed in the same manner as in Example 1. Also, an incubation test was conducted according to Example 1. The results obtained are shown in Table 2.

scarcely reducing sensitivity and gamma. In addition, excellent preservability is shown.

## EXAMPLE 3

A silver halide gelatin photographic emulsion (containing 0.08 mol silver per 100 g) comprising silver bromoiodide containing 1.8 mol percent iodide was prepared by conducting second ripening with the use of the sulfur compound and gold salt in the same manner as in Example 1 and adding 0.4 g, per 1 mol of silver, of polyethylene glycol (mean molecular weight: 2,000) to sensitize the emulsion. The resulting emulsion was divided into three equal portions. One of them was used as a control, and to the remaining 2 portions were added, respectively, the compounds shown in Table 3. Thereafter, film samples were prepared according to Example 1.

Each of the samples was subjected to sensitometry in a known manner to compare the sensitivity, gamma value and fog density, subjected to development at 20°C for 10 minutes in a developer having the following composition, and subsequently processed in the same manner as in Example 1.

|                                |          |
|--------------------------------|----------|
| N-Methyl-p-aminophenol sulfate | 1.5 g    |
| Hydroquinone                   | 1.3 g    |
| Anhydrous sodium sulfite       | 75.0 g   |
| Borax                          | 4.5 g    |
| Potassium bromide              | 0.4 g    |
| Water to make                  | 1 liter. |

30

Also, with respect to each sample, an incubation test was conducted in the same manner as in Example 1. The results are shown in Table 3. It can be seen therein that excellent photographic characteristics can be obtained by the combined use of compound A and compound B.

TABLE 2

| Com-<br>ound | Added<br>amount of<br>compound<br>per 1 mol<br>of silver<br>(mg) | Fresh                        |      |      | Incubated                    |      |      |
|--------------|------------------------------------------------------------------|------------------------------|------|------|------------------------------|------|------|
|              |                                                                  | Relative<br>sensi-<br>tivity | amma | Fog  | Relative<br>sensi-<br>tivity | amma | Fog  |
|              |                                                                  |                              |      |      |                              |      |      |
| Control      | None                                                             | 100                          | 2.85 | 0.06 | 65                           | 2.10 | 0.07 |
| A - 11       | 70                                                               | 75                           | 2.40 | 0.04 | 60                           | 2.10 | 0.06 |
| A - 11       | 140                                                              | 55                           | 2.00 | 0.02 | 45                           | 2.15 | 0.04 |
| A - 11       | 70                                                               | 98                           | 2.80 | 0.03 | 98                           | 2.85 | 0.03 |
| B - 3        | 380                                                              |                              |      |      |                              |      |      |

TABLE 3

| Com-<br>ound | Added<br>amount of<br>compound<br>per 1 mol<br>of silver<br>(mg) | Fresh                        |      |      | Incubated                    |      |      |
|--------------|------------------------------------------------------------------|------------------------------|------|------|------------------------------|------|------|
|              |                                                                  | Relative<br>sensi-<br>tivity | amma | Fog  | Relative<br>sensi-<br>tivity | amma | Fog  |
|              |                                                                  |                              |      |      |                              |      |      |
| Control      | None                                                             | 100                          | 1.08 | 0.17 | 65                           | 0.86 | 0.22 |
| A - 12       | 74                                                               | 65                           | 0.92 | 0.12 | 55                           | 0.75 | 0.15 |
| A - 12       | 74                                                               | 98                           | 1.10 | 0.12 | 101                          | 1.12 | 0.13 |
| B - 5        | 420                                                              |                              |      |      |                              |      |      |

As is clear from Table 2, the combined use of compound A and compound B enables one to remove the defect of the compound A and lowers fogging while

## EXAMPLE 4

A fine-grained silver chlorobromide photographic

emulsion (average grain size was 0.25 microns; containing 0.08 mol silver per 100 g) containing 35 mol percent chloride was prepared and subjected to a second ripening in the same manner as in Example 1. Thereafter, the resulting emulsion was spectrally sensitized by adding the spectrally sensitizing dye represented by the following formula so that sensitization maximum would be at about 555 m $\mu$  (0.1 percent methanol solution of the sensitizing dye was added in

described in "Production of Motion Pictures in Color Using Eastman Color Films," III-15 to III-26, published by Eastman Kodak.

The incubation test was conducted in the same manner as in Example 1. The results obtained are shown in Table 4. Thus, it can be seen that, in a color photographic emulsion also, excellent photographic characteristics can be obtained by the combined use of compound A and compound B.

TABLE 4

| Compound | Added amount of compound per 1 mol of silver (mg) | Fresh                |      | Incubated |                      |
|----------|---------------------------------------------------|----------------------|------|-----------|----------------------|
|          |                                                   | Relative sensitivity | amma | Fog       | Relative sensitivity |
| Control  | None                                              | 100                  | 2.80 | 0.09      | 75                   |
| A - 5    | 34                                                | 62                   | 2.02 | 0.05      | 68                   |
| A - 5    | 34                                                | 98                   | 2.70 | 0.05      | 95                   |
| B - 3    | 680                                               |                      |      |           |                      |

an amount of 8 ml per 100 g of emulsion).



The thus spectrally sensitized emulsion was divided into 3 equal portions. One of them was used as a control. To the remaining 2 portions were added, respectively, the compounds shown in Table 4. Then, a dispersion of gelatin aqueous solution containing dispersed therein as a magenta dye-forming coupler, 1-(2,4,6-trichlorophenyl)-3-[alpha-(2,4-di-t-  
amylphenoxy)-butylamido]benzamido-5-  
pyrazolone(dibutyl phthalate solution) was added to the three emulsions to prepare coating solutions (8 g of magenta coupler per 100 g of emulsion was added). Each of the resulting coating solutions was applied to a cellulose triacetate film support in a coated silver amount of  $9.8 \times 10^{-3}$  mol/m<sup>2</sup>, then dried. The thus prepared samples were subjected to sensitometry in a known manner to compare sensitivity, gamma and fog density. The samples were processed through the processing baths of color development, stop-fixing, bleaching and fixing selected from among the processing steps

25 To fine-grained high contrast silver chlorobrom-iodide emulsions (average grain size was 0.6 microns) containing 1.2 mol percent silver iodide and 8.2 mol percent silver chloride having been subjected to second ripening with the use of the sulfur compound and gold salt in the same manner as in Example 1 were added the compounds described in Table 5, then a dispersion of a gelatin aqueous solution containing dispersed therein as a yellow dye-forming coupler alpha-(2-methoxybenzoyl)-2-chloro-5-[alpha-(2,4-di-t-  
30 amylophenoxy)butylamido]-acetanilide(dibutyl phthalate solution) was added thereto to prepare coating solutions (6.5 g of yellow coupler per 100 g of emulsion was added). The resulting coating solutions were applied to the same paper support as was used in Example 2 in a coated silver amount of  $5.9 \times 10^{-3}$  mol/m<sup>2</sup>, then dried.

35 The thus prepared samples were subjected to sensitometry in a known manner to compare sensitivity, gamma and fog density. The samples were processed according to processing step B for color photographic paper described in Example 2 in U.S. Pat. No. 3,582,322.

An incubation test was conducted in the same manner as in Example 1. The results obtained are shown in Table 5. It can be seen that in this case also fogging alone can be lowered by the combined use of compound A and compound B while maintaining the sensitivity and gamma value, and the photographic characteristics upon storage are extremely stable.

TABLE 5

| Compound | Added amount of compound per 1 mol of silver (mg) | Fresh                |      | Incubated |                      |
|----------|---------------------------------------------------|----------------------|------|-----------|----------------------|
|          |                                                   | Relative sensitivity | amma | Fog       | Relative sensitivity |
| Control  | None                                              | 100                  | 2.43 | 0.12      | 105                  |
| A - 11   | 57                                                | 72                   | 2.15 | 0.08      | 65                   |
| A - 11   | 57                                                | 95                   | 2.40 | 0.08      | 98                   |
| B - 5    | 335                                               |                      |      |           |                      |

While the invention has been described in detail and with reference to specific embodiments thereof, it will be apparent to one skilled in the art that various changes and modifications can be made therein without departing from the spirit and scope thereof.

What is claimed is:

1. A photographic material comprising a support having thereon a silver halide emulsion layer containing (1) at least one of a triazaindene, a tetraazaindene or a pentazaindene having at least one hydroxy group and (2) at least one of a compound having a 1,2-dithiolane ring or a 1,2-dithiane ring represented by the formula:



wherein X represents an alkylene group having 1-6 carbon atoms, R represents a carboxylic acid group, a carboxylic acid salt group, a carboxylic acid ester group, or a carboxylic acid amide group, m represents 2 or 3, and n represents 0 or 1.

2. A photographic material as described in claim 1 wherein said silver halide emulsion is sensitized by at least one chemical sensitizing agent from the group: a sulfur sensitizing agent, a noble metal sensitizing agent, a reduction sensitizing agent or a selenium sensitizing agent.

3. A photographic material as described in claim 1 where the total amount of the (1) at least one of the triazaindene, tetraazaindene and pentazaindene is about 0.005 to about 50 g and the (2) total amount of the at least one of a compound having a 1,2-dithiolane or a 1,2-dithiane ring is about 0.0005 g to 5 g, per 1 mol of silver halide in the silver halide emulsion.

4. A photographic material as described in claim 3 where the total amount of (1) is about 0.05 to 5 g and the total amount of (2) is about 0.0005 to 5 g, per 1 mol of silver halide in the silver halide emulsion.

5. A photographic material as described in claim 1 where in the general formula X is an alkylene group from the series methylene to decylene, when R is an carboxylic acid ester the ester is with a  $C_1 - C_{12}$  alkyl group or a phenyl group and when R is a carboxylic acid amide it is an amide per se or substituted with a  $C_1 - C_{12}$  alkyl group or a phenyl group.

6. A photographic material as described in claim 1 where the triazaindene, tetraazaindene or pentazaindene is substituted with a  $C_1 - C_{17}$  alkyl, aralkyl, aryl,  $C_1 - C_{18}$  alkoxy, carboxyl,  $C_1 - C_{18}$  alkoxy carbonyl, aminocarbonyl, cyano or a group forming a hydrocarbon ring with adjacent carbon atoms in the azaindene ring.

7. A photographic material as described in claim 1 where said compound is



8. A photographic material as described in claim 1 where said compound is



9. A photographic material as described in claim 1 where said compound is



10. A photographic material as described in claim 1 where said azaindene is



11. A photographic material as described in claim 1 where said azaindene is



12. A photographic material as described in claim 1 where said compound is



and said azaindene is



13. A photographic material as described in claim 1 where said compound is



and said azaindene is



14. A photographic material as described in claim 1 where said compound is



and said azaindene is



15. A photographic material as described in claim 1 and said azaindene is where said compound is



5



\* \* \* \* \*

10

15

20

25

30

35

40

45

50

55

60

65